

## UNITED STATES PATENT OFFICE.

HENRY N. DONS, OF ROCHESTER, NEW YORK.

## PROCESS FOR THE MANUFACTURING OF CARBON PAPER FOR USE ON TYPEWRITERS.

No Drawing.

Application filed December 4, 1925. Serial No. 73,267.

- My invention relates to the manufacturing of carbon paper used for typewriting and other purposes. It has been customary to cover the one side of the carbon paper only.
- 5 My invention covers both sides of the paper, one side with coloring matters, oils, fatty acids, waxes, etc., as is usual; and the other side with rosin and black aniline dissolved together in a liquid which evaporates quickly
- 10 such as chloroform, ether, benzine and such liquids, and does not reduce the strength of the paper at the time it is not dry, and passing through the coating machine which any matters dissolved in water will do. This so-
- 15 lution leaves a black sheet which does not give off any color under pressure or in handling, nor does it absorb color from other sheets when dry, and does not leave the side of the paper covered with rosin, black an-
- 20 line and liquid in a state which would be adhesive, which makes it entirely different from a patent formerly issued which patent expressly stipulates that one side was left in an adhesive state.
- 25 According to my process it will be necessary to carry only one color of paper stock, whereas now it is necessary to carry several different colors. Thereby we create an opportunity for a big saving by carrying less
- 30 stock and the elimination of a large amount of waste. It also eliminates special packing for ocean shipments as the paper is fully protected from dampness. This therefore eliminates another big item of expense by
- 35 using rosin and black aniline in solution as stated above, the fibers of which the paper consists are gummed together by the rosin when it is dry, which makes it also waterproof and a great deal stronger. The addition of black aniline makes it possible to use
- 40 paper made of paper stock of mixed colors without sorting or bleaching which would not alone make the paper much cheaper but also stronger as it is a well known fact that the bleaching with chemicals decreases materially the strength of the fiber. The black aniline makes it possible to use the paper stock in its natural color without sorting, as the black aniline is able at all times to produce a uniform satisfactory black color more or less deep according to the amount of aniline used, whereas the other aniline colors, by mixing with the different colors of the paper stock, will produce secondary colors, not satisfactory because on account of the different amounts of colored rags used to produce the paper stock it is impossible to produce from them a product which at all times has the same color, unless it is bleached. It is therefore impossible to state the exact amount of aniline to use in the solution, but the amount of rosin is generally from 8 to 12% compared to the solvent. Shellac either synthetic or natural is preferred but use of other rosins not excluded. It is also possible to use the paper stock mixed with a larger amount of wood pulp because the unbleached fiber is so much stronger than the bleached which is now used.
- 55 What I claim to be new and useful and for which I ask Letters Patent is:
- 60 The process of making carbon transfer paper which consists in coating one side with the usual mixture of wax, fatty acid, oils and coloring material, and the other side with a 65 strengthening composition consisting of aniline-black and rosin dissolved in a volatile solvent, which, because of its quick evaporation, will have no deleterious influence on the paper itself.
- 70
- 75

HENRY N. DONS.